

F. LLOYD.

METHOD OF MAKING HOLLOW METAL RODS.

APPLICATION FILED DEC. 14, 1914.

1,127,041.

Patented Feb. 2, 1915



Witnesses

M. C. Burrell

C. F. Early

Inventor

Frederic Lloyd

By his attorneys

Bailey Wright

# UNITED STATES PATENT OFFICE.

FREDERIC LLOYD, OF SHEFFIELD, ENGLAND.

## METHOD OF MAKING HOLLOW METAL RODS.

1,127,041.

Specification of Letters Patent. Patented Feb. 2, 1915.

Application filed December 12, 1912. Serial No. 874,200.

To all whom it may concern:

Be it known that I, FREDERIC LLOYD, a subject of the King of Great Britain, residing at 26 Alma street, Sheffield, England, have invented new and useful Improvements in Methods of Making Hollow Metal Rods, of which the following is a specification.

In the manufacture of hollow metal rods and the like a central hole is formed in a billet or ingot and sand or similar material is run into the hole and is retained in the hole by plugging its ends. The billet or ingot is then rolled to the required size. It is found in practice that the metal at each end of the billet or ingot is wasted; this waste I have discovered may be prevented if the plugs are dispensed with.

According to this invention the hole in the billet or ingot is completely filled with sand, which is retained in it by metal caps secured to the billet or ingot preferably by welding.

The drawing illustrates a billet or ingot having caps secured to it.

a is the billet having a central hole b and

c c are caps which are secured to the billet and closing the ends of the hole b retain the sand in it. The caps are preferably electrically welded to the billet, and in practice one cap is welded to the billet, and after the hole has been filled with sand the other cap is welded on.

The caps, it will be observed, are applied to the outside only of the billet at opposite ends of the hole and do not project into the hole. After the caps are applied the billet or ingot is rolled or reduced to the required size.

What I claim is:

The herein described method of making a hollow metal rod, which consists in completely filling the hole of a hollow ingot or billet with sand, retaining the sand in the hole by metal caps applied to the outside only of the billet at opposite ends of the hole and then reducing the billet or ingot to the required size.

FREDERIC LLOYD.

Witnesses:

W. PERCY CARPMAEL,  
JOHN H. WHITEHEAD.